

# UNITED STATES PATENT OFFICE.

BRYANT H. BLOOD, OF HARTFORD, CONNECTICUT, ASSIGNOR TO PRATT & WHITNEY COMPANY, OF NEW YORK, N. Y., A CORPORATION OF NEW JERSEY.

## PROCESS OF SEASONING STEEL ARTICLES.

1,373,589.

Specification of Letters Patent.

Patented Apr. 5, 1921.

No Drawing.

Application filed May 13, 1920. Serial No. 381,188.

To all whom it may concern:

Be it known that I, BRYANT H. BLOOD, a citizen of the United States, residing at Hartford, in the county of Hartford and State of Connecticut, have invented certain new and useful Improvements in Processes of Seasoning Steel Articles, of which the following is a specification.

It is a recognized fact that there is a marked tendency for small steel articles which have been hardened to vary in shape or size, either by warping or distortion or by expansion or contraction. Such distortions or variations are ordinarily relatively small and they take place slowly, frequently continuing over a period of months or even of years. For certain classes of work these distortions or variations are so small as to be immaterial, but in work involving high precision the distortions or variations are large enough to seriously interfere with the accuracy required.

Distortions or variations such as above referred to are particularly detrimental in the case of dimension gage blocks which are made with opposite parallel flat end faces at predetermined distances apart, the blocks being furnished in sets with different lengths so that by combining or selecting different blocks any desired dimension within the range of the set can be secured. It is now possible to make blocks of this class so that the maximum error in each block from the nominal size thereof is not more than five millionths of an inch and is frequently as low as one millionth of an inch. When accuracy of this order is attainable the matter of distortion or variation from the form and size of the block as originally made is of vital importance. It has been found that gage blocks that are initially accurate within the limits specified may after a period of some weeks or months have become so distorted or changed in shape or size as to have errors far in excess of the allowable maximum.

It is well known that these distortions or variations gradually diminish in extent, the steel slowly approaching a permanent condition, which condition however may not be fully attained until after a period of months or even of years following hardening. It appears that a certain natural seasoning operation takes place, probably assisted by the

natural changes in temperature to which the steel is subjected by reason of varying weather conditions, and probably further assisted by the shocks and vibrations to which an article is subjected during use.

Ordinarily it is not practical to rely upon this natural seasoning operation because of the long time required and the object of the present invention is to provide a process of seasoning which is capable of securing the same or substantially the same permanency that is secured by natural seasoning but which is capable of being carried out in a relatively short period of time.

In accordance with the invention the steel gage blocks or other articles after having been first made in approximately the desired final forms or sizes are hardened in any usual or preferred way.

The gage blocks or other articles are then placed in an oil bath which is gradually heated to a relatively high temperature. The temperature used is dependent to some extent upon temperatures that have been previously used during hardening and upon the composition of the steel used, but it is ordinarily from 300 to 450° F. In any case it is preferably as high as can be used for the particular steel without softening it to an objectionable extent. The predetermined temperature having been reached the oil with the blocks therein is maintained at this temperature for a definite period, preferably about one to eight hours. For one grade of steel used for gage blocks it has been found that a temperature of 400° maintained for eight hours gives satisfactory results. At the end of the heating period the oil bath with the blocks still therein is allowed to slowly return to normal temperature. After the blocks are removed from the oil bath they are subjected to a large number of alternate dips in hot and cold baths. The hot and cold baths have temperatures respectively somewhat above and below the normal temperature. Preferably the hot bath is of oil, the temperature of which is maintained at about 250 to 285° F. Preferably the cold bath is of kerosene, the temperature of which is maintained at about 0 to -20° F. The blocks are dipped alternately into the hot oil and into the cold oil, being allowed to remain in each long enough to attain the temperature of the

bath throughout. The number of dips in the baths may be varied but I have found that seventy dips in each bath is a desirable number.

5. Under some circumstances it may be desirable or preferable to vibrate the articles during some or all of the before mentioned heat treating steps. Vibration may be effected while the articles are in the initial 10 high temperature bath or while in all of the baths. The vibration is believed to assist the molecules of the metal to rearrange themselves and thus relieve the stresses set up by the hardening operation.

15. The vibration may be effected in any desired way, as, for instance, by mounting the gages or other articles in a suitable frame and by subjecting the frame to the action of a pneumatic hammer.

20. As the result of the foregoing treatment the blocks or other articles have within a short time been caused to undergo those distortions or variations which would otherwise have been distributed over a period of months 25 or years. The blocks or other articles are in substantially permanent form and are ready to be subjected to final grinding or lapping operations whereby they are made accurate within the limits required.

30. What I claim is:

1. The herein described process of seasoning steel articles after hardening, which consists in placing the articles in a liquid bath, slowly heating the bath with the articles 35 to a relatively high temperature, permitting the bath with the articles to slowly cool to normal temperature, and then alternately dipping the articles a large number of times in hot and cold baths at temperatures respectively above and below the normal temperature.

2. The process as described in claim 1 in which the initial bath is heated to a temperature as high as is possible without objectionably softening the steel.

45. The process as described in claim 1 in

which the initial bath is heated to a temperature of from 300 to 450° F.

4. The process as described in claim 1 in which the initial bath is maintained at its 50 maximum temperature for a considerable period of time.

5. The process as described in claim 1 in which the initial bath is maintained at its maximum temperature for a period of from 55 one to eight hours.

6. The process as described in claim 1 in which the temperatures of the hot and cold baths are respectively from 250 to 285° F. and from 0 to -20° F.

60. The process as described in claim 1 in which the articles are dipped approximately seventy times in each of the last said baths.

7. The herein described process of seasoning steel articles after hardening, which consists in placing the articles in a liquid bath, slowly heating the bath with the articles to a temperature from 300 to 450° F., maintaining the bath with the articles at the said temperature for a period of approximately 70 from one to eight hours, permitting the bath with the articles to slowly cool to normal temperature, and then alternately dipping the articles approximately seventy times in hot and cold baths at temperatures respectively from 75 250 to 285° F. and from 0 to -20° F.

9. The process as described in claim 1 in which the articles are vibrated during at least a part of the process steps specified.

80. The process as described in claim 1 in which the articles are vibrated while in the initial high temperature bath.

11. The process as described in claim 1 in which the articles are vibrated while in the 85 low temperature bath.

12. The process as described in claim 1 in which the articles are vibrated while in all of the baths.

In testimony whereof, I hereto affix my 90 signature.

BRYANT H. BLOOD.